

UNITED STATES PATENT OFFICE

2.040.057

## MANUFACTURE OF LUBRICATING OIL

**Robert E. Manley and Howard H. Gross, Beacon,  
N. Y., assignors to The Texas Company, New  
York, N. Y., a corporation of Delaware**

**No Drawing. Application February 25, 1933,  
Serial No. 658,668**

**16 Claims. (Cl. 196—13)**

This invention relates to the manufacture of lubricating oil characterized by a low pour test and having other desirable qualities including a desired green fluorescence.

accomplished by cold settling, filtration, or centrifuging. However, lubricating oil stocks, after dewaxing by these processes, may still retain a substantial amount of wax and, therefore, may have a pour test well above 0° F. The removal of further quantities of wax from these stocks in order to further reduce the pour test necessitates further processing.

On the other hand, the presence of a certain amount of wax in lubricating oils may be beneficial from the standpoint of producing a lubricating oil having a suitable temperature-viscosity characteristic. Consequently, it is of advantage to add to the oil a material which will have the effect of reducing the pour test or cold test to the desired extent without the necessity of entirely removing the remaining wax. 10 15

The material of our invention is simply and readily prepared from oil refinery waste materials by the employment of a procedure comprising 20 treating steps which are more or less similar to those used in ordinary petroleum refining operations.

Waste materials suitable for use in preparing the pour-depressing material of our invention advantageously comprise cracked petroleum tar, sometimes referred to as "pressure-tar", resulting from the liquid or vapor-phase cracking of mineral oil for the production of motor fuels. Other suitable materials may comprise the extract material separated from petroleum fractions, particularly lubricating oil fractions, during the refining of such fractions with solvents such as furfural, liquid sulphur dioxide, and the like. The polymerized material removed from cracked naphtha by treatment with a catalytic adsorbent clay may also be utilized. 25 30 35

We have found that the pour-depressing material produced from these sources in accordance with the procedure of our invention possesses, in addition to its wax crystal inhibiting properties, the ability to impart a desired green fluorescence to lubricating oils which are normally deficient in this respect. 40

The preparation of fluorescent bodies and their 45 beneficial effect when added to lubricating oil fractions is known in the prior art, but such materials heretofore have been prepared from coal tar products or residues which are known to be rich in aromatic bodies or constituents of the 50 desired character.

The raw materials, or oil refinery waste materials from which our product is prepared, do not, in their original condition, contain the desired constituents to any appreciable extent. If pres- 55

ent to any appreciable extent, they are at least not readily recoverable from these waste materials by usual extraction procedures.

- We have found, however, that by subjecting these refinery waste materials to substantial cracking whereby a high melting point pitch is formed, representing about 50% or 60% of the charge, such pitch contains these desired bodies in substantial amount.
- 10 The preparation of these bodies from such waste carbonaceous materials and their addition to lubricating oil stocks will now be described in more detail.

The waste carbonaceous bodies, such as a cracked petroleum tar, or a solvent extract obtained from the solvent refining of mineral oil, is subjected to cracking at temperatures of about 850° to around 1000° F. and under pressures which may range from substantially above atmospheric 15 to 400 pounds or higher. The particular temperatures and pressures employed, as well as the duration of the time to which the material is subjected to cracking conditions, will depend upon the nature of the material, but may advantageously be 20 adjusted or regulated so as to convert the charge into a residue, comprising, for example, about 60% of the charge. This residue, which is in the nature of a pitch, solid at room temperature and having a ball and ring melting point of around 25 160° to 180° F., contains the desired pour-depressing bodies. This pitch from recracked pressure tar or cracked extraction products of the character described is found to be primarily insoluble 30 in mineral lubricating oil, but contains desirable oil-soluble pour depressant constituents in concentrated form. The pitch is particularly free from objectionable oil-soluble material which imparts a darkening effect to pale lubricating oils. 35 This pitch, while maintained in a fluid condition, as, for example, by heating to 200° or 250° F., is mixed with, or dissolved in, a suitable solvent. The solvent advantageously comprises a portion of the lubricating oil stock to which the final pour-depressing and fluorescent material is 40 45 to be added. It may be mixed with this solvent mineral oil fraction in proportions varying from 5 to 50 volumes of pitch to 100 volumes of oil.

To this mixture, a solid adsorbent catalytic material is added, ranging from about 10 pounds to 50 45 pounds per barrel of mixture. The catalytic material may comprise a diatomaceous earth or fuller's earth, or may consist of an acid-treated clay.

The mixture of oil and clay is then heated to 55 temperatures of around 350° to 400° F. in the presence of steam, if desired, and filtered while hot. The catalytic material, during this preceding operation, is believed to exert a polymerizing effect upon the undesired constituents of the extracted material, and which polymerized constituents are removed along with the clay in the form of a filter cake during the filtering operation.

The resulting filtrate contains the desired extracted bodies which, when added to the lubricating oil stock, substantially depress the pour test of the oil as well as impart thereto the desired color characteristics. This filtrate, containing the extract, may then be added to the lubricating oil stock in the proportion of about 4 to 10 60 70 parts of filtrate to about 96 to 90 parts of lubricating oil stock and the whole subjected to mixing.

For example, the addition of about 6 parts of this filtrate to 94 parts of a lubricating oil fraction derived from mixed base crude, having a Saybolt 75 universal viscosity of around 300 seconds at 100°

F. and a pour test of 25° F., reduces the pour test to around 0° F.

While certain temperature and pressure conditions as well as liquid proportions have been set forth in the foregoing example, the invention is not restricted to these particular conditions since they may be varied as desired, depending upon the nature of the materials undergoing treatment.

In accordance with the foregoing procedure, the extracted pour-depressing material is added to lubricating oil stock which has been previously subjected to refining, either by solvent treatment or treatment with acid or other chemicals, followed by contacting with clay. It is contemplated, however, that the high melting point pitch from which the pour-depressing materials are to be extracted may be added directly to the main body of lubricating oil stock before this stock has been subjected to contact filtration in the presence of clay. In this way, only a single contact filtration operation with clay will be necessary.

As already indicated, the pour-depressing and fluorescent bodies dissolved from the high melting point pitch may be separated from the solvent in which they are dissolved in order to produce them in substantially concentrated form. This concentrated material, if desired, may be selectively extracted with solvents of differing solvent capacity, or with relatively light or volatile solvents in order to segregate the material into fractions, some of which may be segregated in a substantially dry or powdery form. It has been found that the material in this latter form may also be added to lubricating oil stocks with equal effect.

Reference to "cracked petroleum tar" in the appended claims includes tarry residues formed during the usual liquid or vapor-phase cracking of mineral oil for the production of motor fuel. The term "extraction products" is intended to include extracted materials and polymerized bodies, as already indicated, which are removed from petroleum fractions including naphtha, kerosene and lubricating oil fractions by extraction with various solvent liquids, or by contacting these fractions with catalytic or other treating agents.

Obviously many modifications and variations of the invention, as hereinbefore set forth, may be made without departing from the spirit and scope thereof, and therefore only such limitations should be imposed as are indicated in the appended claims.

We claim:

1. In the process of manufacturing mineral lubricating oil from lubricating oil stock containing paraffin wax and deficient with respect to color characteristics, the method of reducing the pour test of the oil and imparting thereto a desired green fluorescence which comprises substantially cracking at high temperature and under superatmospheric pressure an oil refinery residue selected from the group consisting of cracked petroleum tar, extraction products separated in the solvent refining of petroleum fractions, and extraction products separated from adsorbent filters in the refining of petroleum fractions to produce a pitch containing constituents having the desired characteristics, dissolving oil-soluble material from the pitch in a portion of the lubricating oil stock to be treated, mixing therewith a comminuted solid adsorbent catalytic material, filtering the mixture to produce a filtrate containing hydrocarbon bodies extracted from the pitch which have the desired pour-depressing and fluorescent characteristics and are

free from undesirable constituents, and mixing said filtrate with the main body of lubricating oil stock to produce a lubricating oil of desired characteristics.

5 2. In the process of manufacturing mineral lubricating oil from lubricating oil stock containing paraffin wax and deficient with respect to color characteristics, the method of reducing the pour test of the oil and imparting thereto the 10 desired green fluorescence which comprises subjecting an oil refinery residue selected from the group consisting of cracked petroleum tar, extraction products separated in the solvent refining of petroleum fractions, and extraction products separated 15 from adsorbent filters in the refining of petroleum fractions to substantial cracking at a temperature of from about 800° F. to around 1000° F. and under superatmospheric pressure to produce a high melting point pitch which is primarily 20 insoluble in mineral lubricating oil but contains oil-soluble constituents having the desired pour-depressing and coloring characteristics, dissolving oil-soluble constituents from the pitch in the lubricating oil stock to be treated, 25 mixing therewith a comminuted solid adsorbent catalytic material, heating the resulting mixture and filtering while hot to produce a filtrate comprising lubricating oil having the desired cold test and fluorescent characteristics and free from 30 undesirable constituents.

3. In the process of manufacturing mineral lubricating oil from lubricating oil stock containing paraffin wax and deficient with respect to color characteristics, the method of reducing the pour test of the oil and imparting thereto the desired green fluorescence which comprises subjecting an oil refinery residue selected from the group consisting of cracked petroleum tar, extraction products separated in the solvent refining of petroleum fractions, and extraction products separated from adsorbent filters in the refining of petroleum fractions to substantial cracking at temperatures of from about 800° F. to around 1000° F. and under superatmospheric pressure to thereby produce a pitch which is primarily insoluble in mineral lubricating oil but contains oil-soluble constituents having the desired pour-depressing and coloring characteristics, dissolving oil-soluble constituents from the pitch in a portion of the lubricating oil stock to be treated, mixing therewith a comminuted acid-treated clay, heating the mixture in the presence of steam to an elevated temperature not substantially exceeding 400° F., filtering while hot to produce a filtrate containing hydrocarbon bodies having the desired characteristics and free from undesirable constituents, and mixing said filtrate with the main body of lubricating oil stock to produce a lubricating oil of desired characteristics.

4. The method of preparing a material adapted to reduce the pour test of mineral lubricating oils and to impart thereto a desired green fluorescence, which comprises subjecting an oil refinery residue selected from the group consisting of cracked petroleum tar, extraction products separated in the solvent refining of petroleum fractions, and extraction products separated from adsorbent filters in the refining of petroleum fractions, to substantial cracking at high temperature and under superatmospheric pressure to form a pitchy residue which is primarily insoluble in mineral lubricating oil but contains oil-soluble constituents having the desired pour-depressing 75 and coloring characteristics, and separating said

constituents from the pitch by extraction with a solvent.

5. The method of preparing a material adapted to reduce the pour test of mineral lubricating oils and to impart thereto a desired green fluorescence, which comprises subjecting an oil refinery residue selected from the group consisting of cracked petroleum tar, extraction products separated in the solvent refining of petroleum fractions, and extraction products separated from adsorbent filters in the refining of petroleum fractions, to substantial cracking at high temperature and under superatmospheric pressure to form a high melting point pitch solid at ordinary temperatures, which is primarily insoluble in mineral lubricating oil but contains oil-soluble constituents having the desired pour-depressing and coloring characteristics, mixing a mineral oil fraction with said pitch adapted to extract said constituents therefrom, heating the resulting mixture to effect extraction, and removing the solvent liquid therefrom to produce the desired material in concentrated form.

6. The method of preparing a material adapted to reduce the pour test of mineral lubricating oils and to impart thereto a desired green fluorescence, which comprises subjecting an oil refinery residue selected from the group consisting of cracked petroleum tar, extraction products separated in the solvent refining of petroleum fractions, and extraction products separated from adsorbent filters in the refining of petroleum fractions, to substantial cracking at high temperature and under superatmospheric pressure to form a pitchy residue which is primarily insoluble in mineral lubricating oil but contains oil-soluble constituents having the desired pour-depressing and coloring characteristics, mixing a lubricating fraction of mineral oil with said residue and commingling therewith a comminuted acid-treated clay, heating the resulting mixture and filtering while hot to remove undesired impurities and produce a filtrate containing the desired material dissolved in the oil.

7. The method of preparing a material adapted to reduce the pour test of mineral lubricating oils and to impart thereto a desired green fluorescence, which comprises subjecting an oil refinery residue selected from the group consisting of cracked petroleum tar, extraction products separated in the solvent refining of petroleum fractions, and extraction products separated from adsorbent filters in the refining of petroleum fractions, to substantial cracking at high temperature and under superatmospheric pressure to form a pitchy residue which is primarily insoluble in mineral lubricating oil but which contains desired oil-soluble pour depressant constituents mixing a lubricating fraction of mineral oil with said residue and commingling therewith a comminuted acid-treated clay, heating the resulting mixture in the presence of steam to an elevated temperature not substantially exceeding 400° F. and filtering while hot to remove undesired impurities and produce a filtrate containing the desired material dissolved in the oil.

8. The method of producing a pour point reducing agent for a mineral lubricating oil, which comprises subjecting an oil refinery residue selected from the group consisting of cracked petroleum tar, extraction products separated in the solvent refining of petroleum fractions, and extraction products separated from adsorbent filters in the refining of petroleum fractions, to substantial cracking at high temperature and

- under superatmospheric pressure to reduce the material to a pitch substantially solid at atmospheric temperatures which is primarily insoluble in mineral lubricating oil but which contains desired oil-soluble pour-depressant constituents.
9. The method of producing a pour point reducing agent for a mineral lubricating oil, which comprises subjecting an oil refinery residue selected from the group consisting of cracked petroleum tar, extraction products separated in the solvent refining of petroleum fractions, and extraction products separated from adsorbent filters in the refining of petroleum fractions, to cracking at temperatures of around 800° to 1000° F. and under superatmospheric pressure to reduce the material to a high melting point pitch representing a residuum in excess of 50% by weight on the weight of the original residue, said pitch being primarily insoluble in mineral lubricating oil but containing desired oil-soluble pour-depressant constituents in concentrated form.
10. The method of producing a pour point reducing agent for a mineral lubricating oil, which comprises subjecting an oil refinery residue consisting of the extraction product separated from adsorbent filters in the clay vapor treating of cracked naphtha to substantial cracking at high temperature and under superatmospheric pressure to reduce the material to a pitch which is primarily insoluble in mineral lubricating oil but which contains desired oil-soluble pour-depressant constituents.
11. The method of producing a pour point reducing agent for a mineral lubricating oil, which comprises subjecting an oil refinery residue consisting of the extraction product separated in the solvent refining of a lubricating oil stock, to substantial cracking at high temperature and under superatmospheric pressure to reduce the material to a pitch which is primarily insoluble in mineral lubricating oil but which contains desired oil-soluble pour-depressant constituents.
12. The method of producing a pour point reducing agent for a mineral lubricating oil, which comprises subjecting pressure tar to re-cracking at high temperature and under superatmospheric pressure to produce a material which is primarily insoluble in mineral lubricating oil in which oil soluble pour point reducing constituents are highly concentrated.
13. A lubricating oil of relatively low pour point comprising a blend of a mineral lubricating oil of relatively higher pour point with a minor proportion of oil-soluble constituents extracted from a pitch which is primarily insoluble in lubricating oil and obtained by cracking an oil refinery residue selected from a group consisting of 10 cracked petroleum tar, extraction products separated in the solvent refining of petroleum fractions, and extraction products separated from adsorbent filters in the refining of petroleum fractions.
14. A lubricating oil of relatively low pour point comprising a blend of a mineral lubricating oil of relatively higher pour point with a minor proportion of a highly concentrated pour point depressant obtained by re-cracking at high temperature and under superatmospheric pressure a pressure tar to a pitchy residue which is primarily insoluble in mineral lubricating oil but in which oil-soluble pour-depressant constituents are highly concentrated.
15. A lubricating oil of relatively low pour point comprising a blend of a mineral lubricating oil of relatively higher pour point with a minor proportion of oil-soluble constituents extracted from a pitch which is primarily insoluble in the 30 lubricating oil and obtained by substantial cracking at high temperature and under superatmospheric pressure of an extraction product separated from adsorbent filters in the clay vapor treating of cracked naphtha.
16. A lubricating oil of relatively low pour point comprising a blend of a mineral lubricating oil of relatively higher pour point with a minor proportion of oil-soluble constituents extracted from a pitch which is primarily insoluble in the 40 lubricating oil and obtained by substantial cracking at high temperature and under superatmospheric pressure of an extraction product separated in the solvent refining of a lubricating oil stock.

45  
ROBERT E. MANLEY.  
HOWARD H. GROSS.

CERTIFICATE OF CORRECTION.

Patent No. 2,040,057.

May 5, 1936.

ROBERT E. MANLEY, ET AL.

It is hereby certified that error appears in the printed specification of the above numbered patent requiring correction as follows: Page 2, second column, line 67, and page 3, first column, lines 16 and 42, claims 1, 2 and 3 respectively, after the word "fractions" insert a comma; page 3, second column, line 58, claim 7, after "constituents" insert a comma; page 4, second column, line 9, claim 13, after "cracking" insert the words at high temperature and under superatmospheric pressure; and that the said Letters Patent should be read with these corrections therein that the same may conform to the record of the case in the Patent Office.

Signed and sealed this 3rd day of November, A. D. 1936.

Henry Van Arsdale

(Seal).

Acting Commissioner of Patents.